

April 11, 1972

R. J. OTT ET AL

3,655,767

FLOW CHARACTERISTICS OF WAXY PETROLEUM RESIDUUM

Original Filed Sept. 20, 1965

FLOW PERFORMANCE OF RANGELY/REDWASH CRUDE BLENDS



ROY J. OTT  
HAROLD N. MILLER INVENTORS

BY *C. B. Barris* PATENT ATTORNEY

1

3,655,767  
FLOW CHARACTERISTICS OF WAXY  
PETROLEUM RESIDUUM

Roy John Ott, Riverdale, N.Y., and Harold Nelson Miller, Millington, N.J., assignors to Esso Research and Engineering Company  
Original application Sept. 20, 1965, Ser. No. 488,707.  
Divided and this application Apr. 25, 1968, Ser. No. 724,245

Int. Cl. C07c 49/76  
U.S. Cl. 260—592

3 Claims

ABSTRACT OF THE DISCLOSURE

A process for preparing blending agents for improving the flow characteristics of high wax-containing oils by adding a C<sub>18</sub>—C<sub>24</sub> carboxylic acid halide-Friedel-Crafts catalyst complex to styrene dissolved in a solvent and simultaneously polymerizing and acylating said styrene monomer.

This is a division of Ser. No. 488,707, filed Sept. 20, 1965 and now abandoned.

This invention is concerned with the preparation and utilization of acyl polystyrenes having C<sub>18</sub>—C<sub>24</sub> acyl side chains attached to the polystyrene nucleus as blending agents for improving flow characteristics of high wax-containing petroleum oils, i.e. crudes, residua, and light fuel oils and especially petroleum oils which boil above 650° F. and have flow points above 75° F.

The pour points of petroleum oils vary widely, for example, some oils freeze far below zero while others are solid up to 80° or 100° F. by virtue of their wax content alone. It is obvious, that the pour point is critical with regard to the flow characteristics and, consequently, the storage, mixing, pumping, etc. of such oil. Thus, pour point characteristics are significant to the design and/or operation of facilities for the storage, heat exchange, pumping, etc. of the oil. Naturally, an oil having a high flow point, e.g. above about 75° F. would provide a serious problem relative to the design of the facilities mentioned above.

Typical examples of petroleum oils which exemplify the undesirable characteristic of having a flow point above about 75° F. are the residual oils set forth in the following Table I:

2

However, while such Zelten residuum typifies the kind of high-wax containing oils which exemplify undesirable flow properties and the like, such residuum is, in fact, a premium oil as compared to other crude residua which have much lower pour points. This fact may be illustrated by a comparison of Zelten waxy oil with crude petroleum residua known as Aramco and Kuwait, as illustrated in the following Table II:

TABLE II.—PROCESSING ZELTEN CRUDES

|    | Volume percent 680° FVT in crude     | Heavy fuel oil inspections |        |        |        |
|----|--------------------------------------|----------------------------|--------|--------|--------|
|    |                                      | Zeiten                     | Aramco | Kuwait | Target |
| 15 | 35                                   | 39                         | 37     |        |        |
| 16 | Inspections on 680° FVT plus:        |                            |        |        |        |
| 17 | Gravity, °API                        | 22                         | 15     | 14     |        |
| 18 | Sulfur, weight percent               | 0.4                        | 3.0    | 4.2    | 1.3.5  |
| 19 | Viscosity, S <sub>1</sub> at 122° F. | 65                         | 110    | 340    | 40-175 |
| 20 | MNI, weight percent                  | 2.3                        | 4.0    | 3.8    | 1.7    |
| 21 | Conradson carbon, weight percent     | 4.5                        | 8-9    | 10-11  |        |
| 22 | Flow point, °F.                      | 105                        | 65     | 55     | 175    |
| 23 | Hot filtration sed., weight percent  | 0.01                       | 0.02   | 0.02   | 1.0.15 |

<sup>1</sup> Maximum.

The inspections shown in the foregoing Table II illustrate that the Zelten residuum is a premium product per se, as well as a valuable product for blending and for improving other heavy fuel oils due to its low sulfur content, low viscosity, low MNI (Modified Naphtha Insolubles), and low Conradson Carbon number. Furthermore, it is low in ash and vanadium content. These qualities also make Zelten crude residuum an excellent cracking stock for obtaining various valuable products, such as straight chain olefins, and the like. As presented, the column headed by the notation "Target" indicates the parameters of blends which are desirable using said Zelten residuum as a blending stock, i.e. providing the flow point can be suitably lowered. For example, it may be desirable to mix the Zelten residuum in a 50/50 mixture with the Aramco or Kuwait residuum. While such blending lowers the wax content, the flow point is generally not sufficiently reduced so as to significantly change the characteristics of the resulting mixture so as to facilitate the handling thereof.

Thus, while it is found that blending of the extremely high wax-containing petroleum residual oils with other

TABLE I.—PETROLEUM RESIDUAL OILS

| Location/Field                 | Column Number |        |        |        |      |      |       |         |                        |                |
|--------------------------------|---------------|--------|--------|--------|------|------|-------|---------|------------------------|----------------|
|                                | 1             | 2      | 3      | 4      | 5    | 6    | 7     | 8       | 9                      | 10             |
|                                | Zelten        | Mabruk | Raguba | Dahra  | Waha | Bomu | Ebubu | Olobiri | Venezuela, San Joaquin | Sumatra, Minas |
| Flow points of residual (° F.) | 105           | 110    | 97     | 99/100 | 85   | +100 | +100  | +100    | +110                   | 115            |
| ° FVT cut point of residual    | +680          | +680   | +650   | 650    | 650  | 650  | 650   | 650     | 650                    | 650            |

While the present invention is directed to substantially all petroleum oils, special reference is made to residual oils boiling above 650° and having a flow point above 75°, with particular reference being made to the residuum of a North African crude identified above as Zelten residuum which contains about 20 weight percent wax. This wax includes waxes of relatively high molecular weight, i.e. from about C<sub>30</sub>—C<sub>50</sub> paraffins which gives rise to a number of the above-mentioned problems, i.e. the transporting, storing, etc. of this kind of heavy oil.

blending stocks may lower the wax content, the flow point cannot be satisfactorily reduced without using the specially adapted C<sub>18</sub>—C<sub>24</sub> acyl polystyrene additives to lower the flow point below the 75° F. target referred to above in Table I. For example, in the 50/50 Zelten/Aramco blend, the addition of only 0.05 weight percent of the C<sub>18</sub>—C<sub>24</sub> acyl polystyrene additive of the instant invention has been found sufficient to meet the target of 75° F. flow point. This advantageous aspect will be discussed more fully herein later.

Furthermore, although Zelten crude or similar petroleum oils or mixtures containing such petroleum oils may have a relatively low viscosity as measured by conventional methods as compared to heavy oils of low wax content, the handling of the high wax content residuum creates special difficulties which are due to the manner in which the oil undergoes changes in flow characteristics on being subjected to changes in temperature. Generally, the standardized ASTM pour point is reasonably indicative of how low the temperature of an oil can be decreased and at what point it can be satisfactorily made to flow. However, with high waxy residua, such as the above-described Zelten Oil, the flow point determined by standardized procedure is variable and is further, a function of prior thermal treatment.

This phenomena may be referred to as a "pour gap" and is determined when high waxy residua in the presence of natural pour depressants or certain synthetic pour depressants exhibit pour reversion. This is determined by subjecting a mixture of residuum and pour depressant through a series of heating and reheating cycles so as to determine the various pour points at reheat temperatures. The following Table III illustrates the effects of various known additives on the various pour points at reheat temperatures and, consequently, the flow point of Zelten residuum.

TABLE III.—EFFECTS OF ADDITIVES ON FLOW POINTS OF 680° F. PLUS VIRGIN ZELTEN RESIDUUM

| Additive                            | Concen-<br>tration | ° F. pour points at reheat temperature<br>(TRH = ° F.) |     |     |     |     |     | Averages<br>of number<br>of tests | Flow<br>point <sup>1</sup> | Pour<br>gap |
|-------------------------------------|--------------------|--------------------------------------------------------|-----|-----|-----|-----|-----|-----------------------------------|----------------------------|-------------|
|                                     |                    | 100                                                    | 115 | 130 | 150 | 180 | 200 |                                   |                            |             |
| 680° F. plus virgin Zelten residuum | 1.00               | 100                                                    | 105 | 105 | 100 | 95  | (3) | 105                               | 105                        | 10          |
| Wax-phenol (ex. 180 m.p. wax)       | 0.30               | 90                                                     | 97  | 102 | 110 | 85  | 60  | (2)                               | 110                        | 50          |
| Wax-naphthalene (ex. 180 m.p. wax)  | 0.30               | 83                                                     | 99  | 109 | 103 | 100 | 65  | (4)                               | 109                        | 44          |
| Wax-naphthalene (ex. 150 m.p. wax)  | 0.30               | 98                                                     | 103 | 105 | 105 | 109 | 90  | (4)                               | 109                        | 19          |
| Target pour points                  |                    | 75                                                     | 75  | 75  | 75  | 75  | 75  |                                   | 75                         |             |

<sup>1</sup> Flow point—maximum pour point obtained after a series of pour point determinations at a series of reheat temperatures.

It is apparent from the foregoing table that; conventional pour depressants fail to suitably reduce the flow point of the residuum inasmuch as reheating through one or more temperature cycles results in at least one pour point which would be essentially inoperable for commercial handling of the residuum. Thus, the necessity for a suitable additive which will effectively reduce the flow point of high waxy residua through any number of reheat cycles is readily apparent.

In addition, from the foregoing Table III it is apparently necessary to modify the standard ASTM pour point procedure so as to obtain a reproducible and more meaningful measure of flow characteristics and to efficiently test the high wax-containing residual oils. Accordingly, in the tests illustrated in the flow point test of Table III, a sample of oil is first heated to 200° F. and is subsequently cooled to 32° F. before it is again heated to an intermediate temperature in the range of 90° to 200° F. for testing under the standard ASTM procedure. By putting the oil through a temperature cycle series, such as mentioned above, a determination is made of the "pour gap" as well as the "flow point" corresponding to the maximum pour point in the series. Such flow point is the optimum measure achieved as yet for determining how well such oil can be kept fluid in storage, for pumping, transporting, and the like.

It is accordingly, an object of the present invention to provide an additive which substantially improves the flow characteristics of high wax-containing petroleum oils.

It is also an object of the present invention to provide improved C<sub>18</sub>—C<sub>24</sub> acyl polystyrenes which effectively serve to improve the flow characteristics of extremely high wax-containing petroleum oils such as crudes, residua and light fuel oils that have pour or flow points above 20° F.

It is a special object of the present invention to prepare superior polystyrenes having C<sub>18</sub>—C<sub>24</sub> acyl side chains attached to the polystyrene nucleus as blending agents for improving the flow characteristics of extremely high wax-

containing petroleum residual oils that boil above 650° F. and have pour or flow points above 75° F.

Other objects and advantages will become apparent to one skilled in the art upon a further reading of the following description of the present invention.

Accordingly, the present invention is directed to a petroleum oil composition having improved flow characteristics, which comprises essentially a high wax content petroleum oil, e.g. an oil having a flow point or pour point above 20° F. and especially a residual oil that boils above about 650° F. and has a flow point above about 75° F. improved with respect to its flow characteristics by incorporating and blending therewith an amount of about 0.01 to about 5.0 wt. percent of a C<sub>18</sub>—C<sub>24</sub> polystyrene having the following general formula:



20  
25

25

wherein R is a C<sub>17</sub>—C<sub>23</sub> alkyl group, and the subscript n is a number from 2 to 50 of the recurring unit in the acyl polystyrene.

Specifically, the present invention is predicated on the discovery that the potency of the C<sub>18</sub>—C<sub>24</sub> polystyrenes are remarkably improved with respect to their effect on the flow characteristics of extremely high wax-containing petroleum oils when said polystyrenes are prepared by a process comprising the steps of: (1) forming a complex of an acylating acid halide with a Friedel-Crafts catalyst, (2) gradually adding said complex, either continuously or in sequential portions, to a solution of styrene monomer and, (3) simultaneously acylating and polymerizing the addition mixture.

The above-described sequence of steps differs from the method heretofore employed to form acyl polystyrenes. This known method comprises degrading commercial polystyrene dissolved in an inert solvent, such as ortho-dichlorobenzene, with a Friedel-Crafts catalyst, e.g., aluminum chloride, and adding to this solution from about 0.5 to 1.0 mole of a carboxylic acid halide-Friedel-Crafts catalyst complex per styrene nucleus present. After all the acid halide-Friedel-Crafts catalyst complex has been added to the solution of the polystyrene and the evolution of hydrogen halide has stopped, the catalyst is destroyed by addition of water or alcohol to the reaction mixture. The acylated polystyrene product is then taken up in a suitable hydrocarbon solvent, such as heptane or kerosene, and washed with an aqueous alkaline solution and water. The solvent may be evaporated to isolate the polymer or the polymer may be dissolved in the solvent before blending with the residual oil.

Basically, the sole similarity of the process of the present invention with that of the prior art is the carboxylic acid halide-Friedel-Crafts catalyst complex employed in each process. This complex is formed by mixing and reacting a C<sub>18</sub>—C<sub>24</sub> carboxylic acid halide, e.g. an acid chloride,

with the Friedel-Crafts catalyst, e.g., aluminum chloride, which reaction may be represented as follows:



The components of the above reaction are employed in molar ratios ranging from about 0.9 to 1.1 moles of carboxylic acid halide per mole of Friedel-Crafts catalyst and are preferably employed in equimolar amounts. The complex is formed in the presence of a solvent which will dissolve the components and be unreactive with the components and the resulting complex. Typical solvents include, for example, cyclopentane, cyclohexane, the n-paraffins, ethylene dichloride, nitromethane, nitrobenzene, orthodichlorobenzene, and the like. The reaction is complete in from 15 to 90 minutes when temperatures of from 20° to 70° C. and preferably 20° to 35° C. are employed. The pressure in the reaction zone is not critical and may be varied. Agitation is found to benefit the rate of reaction between the components.

The carboxylic acid halide reactants which are of particular interest and used in the process of the present invention are the C<sub>20</sub> and C<sub>22</sub> acid halides, or mixtures thereof. The halides include chlorides, bromides, fluoride, etc., but the chlorides are preferred. These two acid chlorides which are obtained from straight chain carboxylic acids, such as arachidic and behenic acid, or commercial acid mixtures including these two are preferred. The acid halides may be prepared by treating the corresponding acid dissolved in a suitable inert solvent, such as those hereinbefore set forth, and the like, with halogenating agents such as phosphorus trichloride, thionylchloride, and the like. Reaction temperatures are maintained within the range of from about 20° to about 80° C. and preferably from 45° to 55° C. and pressures may be varied within a wide, non-critical range.

The Friedel-Crafts catalyst used may be any of this well known type of catalyst such as AlCl<sub>3</sub>, AlBr<sub>3</sub>, AlBr<sub>2</sub>Cl, AlClBr<sub>2</sub>, Al<sub>2</sub>Br<sub>5</sub>Cl, AlBr<sub>2</sub>OH·AlBr<sub>3</sub>AlBr<sub>2</sub>, BF<sub>3</sub>, and the like. Aluminum chloride (AlCl<sub>3</sub>) is the preferred catalyst component employed.

The styrene monomer suitably employed in the present invention may comprise any commercial grade styrene monomer, i.e. a styrene monomer having a purity of about 90% or more. It is preferable, however, to employ a styrene monomer having a purity greater than 95%. It is within the purview of the present invention, however, to employ styrene monomer which contains relatively, small amounts of by-product, e.g. less than 5 wt. percent of styrenes having alkyl groups substituted on the ring, e.g., paramethyl styrene, dimethylstyrene, and the like.

In accordance with the present invention, the acid halide-Friedel-Crafts catalyst complex is gradually added to a styrene monomer solution in order to effect simultaneous acylation and polymerization reactions. This reaction may be represented as follows:



In effecting the above-illustrated reaction, the styrene monomer utilized is initially dissolved in a solvent to form a 10 to 90 wt. percent solution, preferably a 20 to 50 wt. percent solution. The solvent must be unreactive with the styrene monomer as well as the acid halide-Friedel-Crafts complex and preferably is a solvent similar to that employed in the acid halide-catalyst complex, for example, cyclopentane, cyclohexane, the n-paraffins, ethylene dichloride, nitromethane, nitrobenzene, orthodichlorobenzene, and the like.

In accordance with the invention, the acid halide-Friedel-Crafts catalyst complex is gradually added to the styrene monomer solution, either continuously or in a plurality of sequential portions. The total polymerization and acylation reaction period will generally range from about 1/2 to 12 hours and in order to prepare the potent additives of the present invention, addition of the acid halide-Friedel-Crafts complex is made over a period of from 3/4 to 4 hours, preferably, 2 to 3 hours. As disclosed, the complex addition may be effected either continuously during the defined addition period or may be added in from about 4 to 100 portions which are added sequentially.

The temperature limitations upon the process of this invention are varied. Broadly, the temperatures range from -25° C. to 100° C. and preferably from 0° C. to 60° C. Although there is both polymerization and acylation reaction during the initial stages of the process, polymerization of the styrene monomer is principal. During the initial stages, therefore, the temperature of the reaction mixture is adjusted so as to obtain the desired degree of polymerization. In order to allow a greater degree of polymerization and a consequent higher molecular weight of product, the reaction temperature is initially maintained to one within the range of from -25° C. to 60° C., preferably 0° to 50° C. In the latter stages of the reaction, wherein the acylation reaction principally occurs, the temperatures should be allowed to rise from the temperature of the initial stage so as to be maintained within the range of from 25° to 100° C., preferably 25° to 60° C. The pressure in the reaction zone is not critical and may be varied within the wide limits. Generally, however, it will be found that atmospheric pressure is quite suitable for carrying out the reaction.

The proportions of the constituents of the reaction mixture may be varied widely, e.g., from about 0.5 to 1.0 mole of acid halide-Friedel-Crafts catalyst complex may be employed per mole of styrene monomer. Preferably, the invention contemplates the use of equimolar proportions of the acid halide-Friedel-Crafts catalyst complex and the styrene monomer.

Reaction of the acid halide-Friedel-Crafts catalyst complex with the styrene monomer results in a complex consisting of acyl polystyrene and Friedel-Crafts catalyst. In order to prepare the additives of the present invention, therefore, this reaction complex is hydrolyzed. This may be represented as follows:





The final product of this invention may be blended directly with the high wax-containing petroleum oils. Concentrations within the range of from 0.01% to 5% by weight of the additive material in the petroleum oils will be operable and will give the desired improvement in flow characteristics. Based on economic as well as flow modifying reasons, from about 0.025 to 0.25 wt. percent of the additive is preferably employed.

The additives of this invention are found compatible with other additive materials and may be blended successfully with petroleum oils containing minor amounts of viscosity index improvers, rust inhibitors, oiliness agents, oxidation inhibitors and the like.

The superior additives of the present invention may be understood more fully from the following examples illustrating same.

#### EXAMPLE I

This example serves to illustrate the preparation of a C<sub>20</sub>-C<sub>22</sub> acyl polystyrene in accordance with the method of the present invention.

A C<sub>20</sub>-C<sub>22</sub> acid chloride-aluminum chloride complex was prepared by adding 40.0 grams of cyclohexane to 72.0 grams of the acid chloride (90% C<sub>20</sub>-C<sub>22</sub>) with agitation. To the resulting mixture was added 28.0 grams of AlCl<sub>3</sub> with agitation. The reaction mixture was maintained in the range of from 22 to 33° C. for a period of 1 hour.

The styrene monomer to be polymerized and acylated was prepared by dissolving 21.0 grams of styrene monomer in 80.0 grams of cyclohexane while maintaining the temperature of the reaction vessel at approximately 25° C. The acid chloride-AlCl<sub>3</sub> complex prepared above was gradually added to the styrene-cyclohexane solution continuously over a period of 2½ hours. During the addition of complex to the styrene solution the reaction temperature increased from 25° C. to 50° C. After addition of the acid chloride-AlCl<sub>3</sub> complex to the styrene monomer solution was completed, the reaction was continued for an additional three hour period while maintaining the temperature of the reaction mixture at approximately 50° C.

The C<sub>20</sub>-C<sub>22</sub> acyl polystyrene was recovered by hydrolyzing the reaction product with about 200 ml. of a mixture containing about 75% water, 15% isopropanol and 10% hydrochloric acid. Hydrolysis was effected with agitation at a temperature in the range of about 100°-150° F. After the evolution of hydrogen chloride ceased, the mixture was allowed to settle for about ½ hour without agitation and the bottom layer was drawn off. This hydrolyzed product was then washed with 200 ml. portions of a water-isopropanol mixture (about 80% water) until the product attained a neutral pH. The C<sub>20</sub>-C<sub>22</sub> acyl polystyrene was then heated under vacuum to 210° F. in order to drive off the volatiles and isolate the product. The yield (dialysis residue) was 88% high molecular weight polymeric product as measured by dialysis.

#### EXAMPLE II

The following example illustrates the adverse effect on the yield of high molecular weight polymeric product which results when the sequence of steps necessary to the present invention are not adhered to.

Four hundred and twenty three pounds of a commercially available mixture of arachidic and behenic acids (C<sub>20</sub> and C<sub>22</sub> acids) and 181 pounds of n-heptene were charged to a 300 gallon glass-lined reactor. The slurry

was stirred, heated to 50° C., and 66.6 pounds (slight excess) of phosphorus trichloride added continuously over 20 to 30 minutes. The reaction mixture was stirred for 11 hours at 50° C., and then allowed to stand 9 hours (overnight) at 50° C., to permit the phosphorus acid to settle. The phosphorus acid was drained from the reactor and the excess PCl<sub>3</sub> distilled overhead at 50° C., under partial vacuum.

The above acid chloride-n-heptane solution was cooled to about 28° C., and 167.0 pounds of aluminum chloride was added portion-wise, while stirring, over ½-1 hour. The reaction mixture was stirred an additional hour to complete the formation of the hydrocarbon soluble complex.

A solution of 130.7 pounds of styrene monomer and 130.7 pounds of n-heptane was added continuously over a period of about 2 hours to the above acid chloride-aluminum chloride complex. The reaction is instantaneous and is indicated by a change in color (to red-orange), by the evolution of copious amounts of gaseous HCl, and by a rapid rise in temperature (highly exothermic). The temperature was permitted to rise to 50° C., and maintained at 50° C., by external cooling. After the styrene addition was completed the reaction was stirred an additional 2 hours at 50° C.

The reaction product was hydrolyzed by adding it to 57 gallons of 10% hydrochloric acid solution and 10 gallons of isopropyl alcohol. The aluminum salt containing acid-water layer was discarded and the organic phase was washed again with dilute HCl followed by 3 clear water washes. The solvent (n-heptane) and residual water were initially stripped out at elevated temperatures under atmospheric pressure and finally completely stripped under vacuum. The yield of active product was less than 65%. This yield represents a difference in yield of active high molecular weight polymeric product of 23% when compared with Example I.

#### EXAMPLE III

Acyl polystyrenes made by the process of the present invention as illustrated in Example I and made by a process outside the scope of the present invention, i.e., wherein the order of addition of components and the manner of same is modified, were compared in order to illustrate the vastly improved potency of the additives of this invention. In the following table various reheat temperature cycles were employed as hereinbefore described in order to test the effectiveness of the additives. Such temperature cycles as well as the additive concentration employed are set forth in Table IV. The residual oil employed was Brega residuum which initially boils at a temperature of about 650° F. and has a flow point of 105° F.

TABLE IV

| 55          | Additive <sup>1</sup> concentration, percent | Pour point at reheat temperature TRH, ° F. |     |     |     |     |     |
|-------------|----------------------------------------------|--------------------------------------------|-----|-----|-----|-----|-----|
|             |                                              | TRH = 200                                  | 180 | 150 | 120 | 115 | 100 |
| Run number: |                                              |                                            |     |     |     |     |     |
| 60          | 1 <sup>2</sup> -----                         | 0.10                                       | 50  | 65  | 70  | 70  | 60  |
|             | 2 <sup>2</sup> -----                         | 0.10                                       | 65  | 75  | 80  | 80  | 65  |
|             | 3 <sup>2</sup> -----                         | 0.10                                       | 40  | 60  | 70  | 80  | 65  |
|             | 4 <sup>2</sup> -----                         | 0.10                                       | 45  | 65  | 50  | 50  | 60  |
|             | 5 <sup>3</sup> -----                         | 0.10                                       | 75  | 85  | 90  | 95  | 75  |
|             | 6 <sup>3</sup> -----                         | 0.20                                       | 75  | 75  | 85  | 75  | 70  |
|             | 7 <sup>3</sup> -----                         | 0.30                                       | 65  | 70  | 70  | 65  | 65  |

<sup>1</sup> Additive concentration in Brega residuum.

<sup>2</sup> Made by process described in Example I.

<sup>3</sup> Made by the process described in Example II.

As will be apparent from an examination of the comparative data reported in Table IV above, the products of this invention impart a three-fold improvement in the flow characteristics of the residual oil with which they are blended. In other words it took three times the concentration (0.3%) of prior art additive to equal the effectiveness of the additive of the instant invention. The economic advantages accruing from this improvement

are readily apparent and need not, it is believed, be further commented on.

#### EXAMPLE IV

FIG. 1 represents comparative data resulting from tests which simulated the handling of high waxy crudes in a pipeline.

The effect of various additives on blends of two specific crude stocks is presented, i.e., Redwash crude from Utah and Rangely crude from Western Colorado. The improvement resulting from the additives of the present invention is readily apparent from said FIG. 1 wherein typical data is set forth in graphical form.

In the various runs, kinematic viscosities at 32° F. were determined with the Burrell-Severs extrusion viscometer. In this test, 50/50 and 65/35 ratios of Rangely/Redwash crude mixtures were placed in the sample reservoir of the viscometer and subjected to various nitrogen pressures represented as the axis of abscissas in the graph of FIG. 1. The capillary diameter of the sample reservoir was 0.074 inch. The resulting flow viscosities, i.e., capillary flow, is presented as the axis of ordinates of said graph. The test temperature utilized, i.e., 32° F. is considered representative of winter operations in an unheated, underground pipeline.

Curves 1A and 1B represent the kinematic viscosities of the blends containing no additives. Curves 2A and 2B represent the kinematic viscosities of blends which contain 0.05 wt. percent of an additive produced in a manner similar to that of Example II, that is, an additive produced by a sequence of steps outside the scope of the present invention. Curves 3A and 3B represent the kinematic viscosities of blends which contain 0.05 wt. percent of an additive similar to that produced in Example I, that is, an acylated polystyrene of the present invention.

From an inspection of the graphical representation of FIG. 1, it is readily apparent that use of the additives of the instant invention results in a remarkable improvement in the full viscosities of crudes under conditions representative of winter operations.

#### EXAMPLE V

Acyl polystyrenes prepared by the process of the present invention, for example, by the process of Example I, and made by a process outside the scope of the present invention, for example, according to Example II wherein the order of addition of components, etc., is modified may also be compared employing light fuel oils or other similar petroleum oils. Upon comparison, it is found that similar beneficial results as hereinbefore illustrated were also encountered with light fuel oils.

In this comparison, three identical 50 ton tanks were filled with about 40 tons each of 200 sec. Light Fuel Oil ex Esso (Karlsruhe) of 65° F. pour-point. All tanks were equipped with 3 thermocouples. The tanks could be heated by a "heating-bell" positioned at the bottom thereof. The tank inlet and offtake was via a telescopic stand pipe in the tank bottom.

The fuel in Tank 1 was left undisturbed for the duration of the test (about 4 months). Upper pour points were carried out on one sample each week. Tanks 2 and 3 were left undisturbed for 3 weeks, then heated to 160° F. for one day, and then left undisturbed for a further 3 weeks. This cycle was repeated 5 times. During the 5th heating cycle 0.05 wt. percent of each of the acylated polystyrene additives, respectively, were blended in (after first cutting

it back with 3-4 times its own weight of kerosene). The tank contents were recirculated for 2 hours to ensure good mixing. Samples were taken during the test period and the pour point determined. The results were as follows:

TABLE V

|    |                                    | Upper pour point ° F. |        |        |
|----|------------------------------------|-----------------------|--------|--------|
|    |                                    | Tank 1                | Tank 2 | Tank 4 |
| 10 | Heat cycle additive.....           | None                  | (1)    | (2)    |
|    | Pour point:                        |                       |        |        |
|    | Initial.....                       | 65                    | 65     | 65     |
|    | Before blending <sup>3</sup> ..... | 65                    | 65     | 65     |
|    | After blending <sup>4</sup> .....  | 65                    | 15     | 50     |
|    | Final <sup>5</sup> .....           | 65                    | 15     | 60     |

<sup>1</sup> To 160° F. every 3 weeks, instant invention (Example I).

<sup>2</sup> To 160° F. every 3 weeks, prior art (Example II).

<sup>3</sup> Before heating.

<sup>4</sup> After blending 0.05 weight percent into Tanks 2 and 3.

<sup>5</sup> 3 weeks after blending.

From the foregoing it can be concluded that the acylated polystyrene additive prepared in accordance with the present invention very effectively improves the flow characteristics of light fuel oils. In addition, no indications of pour point regression occurred in the 3 weeks during which the fuel was stored after the additive of this invention was added.

It is not intended that this invention be limited to the specific examples presented by way of illustration. The scope of the invention is limited only by the appended claims.

What is claimed is:

1. A process for the manufacture of an acyl polystyrene blending agent for improving the flow characteristics of high wax-containing petroleum oils which comprises admixing styrene and an inert solvent for said styrene, gradually adding to the resulting mixture a C<sub>18</sub>-C<sub>24</sub> carboxylic acid halide-Friedel-Crafts catalyst complex over a period of from about 1/4 to 4 hours and simultaneously polymerizing and acylating said styrene monomer at a temperature within the range of from -25° to 100° C. for a total period of time ranging from about 1/2 to 12 hours and recovering said acyl polystyrene.

2. The process according to claim 1 wherein the complex added is a C<sub>20</sub>-C<sub>22</sub> carboxylic acid chloride-aluminum chloride complex and said complex is added continuously over a period of from about 2 to 3 hours.

3. A process for the manufacture of a blending agent for improving the flow characteristics of extremely high wax-containing petroleum residual oils which boil above 650° F. and have a flow point above 75° F. which comprises forming a solution of styrene monomer in an inert hydrocarbon solvent, gradually adding to said solution over a period of from 1/4 to 4 hours and at a temperature of from about 0° to about 50° C., an equimolar portion of a complex formed by admixing substantially equimolar proportions of a Friedel-Crafts catalyst and a C<sub>18</sub>-C<sub>24</sub> carboxylic acid chloride and after said addition simultaneously polymerizing and acylating said styrene monomer at a temperature of from about 25° to 60° C. for a total period of time ranging from 1/2 to 12 hours, and thereafter hydrolyzing the resulting complex formed.

#### References Cited

#### UNITED STATES PATENTS

3,248,186 4/1966 Brownawell et al. 44-62

DANIEL D. HORWITZ, Primary Examiner